

1

3,449,459

LUBRICATING COMPOSITIONS FOR  
COMPRESSION REFRIGERATORS

Michel Asfazadourian, Robert Muths, and Marcel  
Prillieux, Mont-Saint-Aignan, France, assignors to  
Esso Research and Engineering Company, a cor-  
poration of Delaware

No Drawing. Filed Nov. 2, 1966, Ser. No. 591,407  
Int. Cl. C07c 15/02; C09k 3/02

U.S. Cl. 260—671

7 Claims

ABSTRACT OF THE DISCLOSURE

A hydrocarbon lubricating oil that is miscible with a fluorochlorinated hydrocarbon refrigerant at low temperatures is prepared by alkylating, with an olefin polymer such as the trimer, tetramer, or pentamer of propylene, an alkyl benzene having a plurality of short alkyl chains such as methyl ethyl benzene or trimethyl benzene. Preferably, mixtures of such alkyl benzenes are used, as for example a mixture of methyl ethyl benzene and tetra-methyl benzene.

The present invention is concerned with synthetic lubricants intended for the lubrication of compression refrigeration apparatus. These lubricating compositions are characterised by their miscibility with halogenated refrigerating fluids such as the fluorochlorinated hydrocarbons of the "Freon" type.

Synthetic oils obtained by the fractional distillation of the alkylation products of benzene by olefins, in the presence of a Friedel and Crafts catalyst are known; these oils are in fact miscible with refrigerating liquids of the Freon type down to very low temperatures.

The applicants have discovered that alkylated aromatic hydrocarbons, when subjected to superalkylation, furnish products that can be used as lubricating oils for compression refrigerating apparatus.

The alkylaromatic hydrocarbons intended to be superalkylated according to the invention are those having from 1 to 5, and preferably 2 to 3 straight or branched aliphatic chains. Each chain preferably has from 1 to 15 carbon atoms.

Suitable examples are methylethylbenzene, dimethyl-ethylbenzene, trimethylbenzene, tetramethylbenzene, or mixtures of these substances, preferably:

The product known in the trade by the name of Solvesso 100, i.e. a mixture containing 92% methylethylbenzene and tetramethylbenzene and having as its characteristics:

Density ----- 0.872

ASTM distillation:

Initial point ----- °C 158 55  
50% distilled ----- °C 163  
Final point ----- °C 171

Mean molecular weight ----- 120

The product known in the trade as Solvesso 150, a mixture containing 70% dimethylethylbenzene and tetra-methylbenzene and having the following characteristics:

Density ----- 0.892

ASTM distillation:

Initial point ----- °C 187 65  
50% distilled ----- °C 193  
Final point ----- °C 212

Mean molecular weight ----- 135

The petroleum fraction distilling between 170° C. and 325° C., 50% distilled at 181° C., with a mean molecular weight of 136 and a density of 0.905.

2

According to the invention this superalkylation takes place in the presence of a classic alkylation catalyst with olefin polymers, for example a trimer, tetramer or pentamer of propylene and for preference those complying with the following characteristics:

Propylene trimer:

|                             |       |
|-----------------------------|-------|
| Density -----               | 0.740 |
| ASTM distillation:          |       |
| Initial point ----- °C      | 125   |
| Final point ----- °C        | 145   |
| Mean molecular weight ----- | 127   |

Propylene tetramer:

|                             |       |
|-----------------------------|-------|
| Density -----               | 0.777 |
| ASTM distillation:          |       |
| Initial point ----- °C      | 183   |
| 50% distilled ----- °C      | 188   |
| Final point ----- °C        | 222   |
| Mean molecular weight ----- | 172   |

Propylene pentamer:

|                             |       |
|-----------------------------|-------|
| Density -----               | 0.802 |
| ASTM distillation:          |       |
| Initial point ----- °C      | 269   |
| 50% distilled ----- °C      | 271   |
| Final point ----- °C        | 303   |
| Mean molecular weight ----- | 245   |

Suitable alkylation catalysts are sulphuric acid or acids of the Lewis type such as  $\text{AlCl}_3$  or  $\text{BF}_3$ .

Alkylation is performed at a temperature of 0 to 60° C. and preferably at about 40° C. the weight ratio aromatic hydrocarbon/olefin polymer being between 7/1 and 1/1, and preferably between 3/1 and 5/1. The catalyst represents 3 to 10% and preferably 5 to 6% by weight of olefin. The operation takes about one hour.

The lubricating oils according to the invention make it possible to prepare mixtures with halogenated refrigerating fluids, such as the fluorochlorinated hydrocarbons of the "Freon" type, the proportion of lubricant being preferably 1 to 10% by weight of the mixture.

The following example illustrates the invention.

EXAMPLE

Solvesso 100 and Solvesso 150 were superalkylated with propylene tetramer, these substances having the properties mentioned previously. This superalkylation was performed under the following conditions:

Temperature—40° C.

Weight ratio Solvesso/tetrapropylene—5/1.

Catalyst  $\text{AlCl}_3$ —6% by weight of tetrapropylene.

Time—1 hour.

The superalkylated Solvesso 100 had the following characteristics:

|                       |         |
|-----------------------|---------|
| Density -----         | 0.884   |
| Distillation ----- °C | 305/350 |

and the superalkylated Solvesso 150:

|                       |       |
|-----------------------|-------|
| Density -----         | 0.935 |
| Distillation ----- °C | 330   |

Two mixtures M1 and M2 were prepared. Mixture M1 comprised: 35% by volume of superalkylated Solvesso 100; and 65% by volume of superalkylated Solvesso 150. Mixture M2 comprised: 40% by volume superalkylated Solvesso 100; and 60% by volume superalkylated Solvesso 150.

The characteristics of mixtures M1 and M2 were determined according to the following methods:

|                          |                |
|--------------------------|----------------|
| Flash point, open vessel | NFT 60-103     |
| Density                  | NFT 60-101     |
| Cloud point              | ASTM D 97-57   |
| Aniline point            | ASTM D 611-63T |
| Viscosity                | NFT 60-100     |

The following results were obtained:

|                                                | M1    | M2    |
|------------------------------------------------|-------|-------|
| Density, 15° C.                                | 0.906 | 0.896 |
| Flash point open vessel                        | 168   | 160   |
| Viscosity in centistokes at 37.8° C. (100° F.) | 40.0  | 21.9  |
| ASTM colour                                    | 3     | ----- |
| Flocculation point ° C.1                       | < -60 | -37   |
| Cloud point, ° C.                              | -33   | -36   |
| Aniline point, ° C.                            | 35    | 32.5  |

<sup>1</sup> This temperature is that at which precipitation by flocculation takes place in a mixture of 10% lubricating oil and 90% refrigerating fluid. It is ascertained under the following conditions: 1 cc. of the oil to be tested is placed in a thick glass tube; it is then heated to 120° C. and dry nitrogen is injected through the sample for about 10 minutes. The tube is then allowed to cool to the ambient temperature and is placed in a cooling bath, whose temperature is higher by about 8.5° C. than the assumed flocculation point. There are then added 9 cc. Freon 12 (CCl<sub>2</sub>F<sub>2</sub>) and the tube is closed. After checking the homogeneity of the mixture, the tube is put back in the cooling bath and the temperature is lowered by 2.8° C. in 4 minutes and the appearance of the mixture is examined after 15 minutes at this temperature. The process is continued as long as is necessary by lowering the temperature of the bath by fractions of 2.8° C. until the presence is noted of a definite precipitate in the sample. The corresponding temperature of the bath is that of the flocculation point.

It thus appears that the viscosity and the flocculation point can be ascertained by varying the relative proportions of the different superalkylated Solvessos used. The mixture M1 furnishes a particularly interesting flocculation point.

It is obvious that the present invention has been described purely by way of explanation and in no sense restrictively and that any modifications may be made to it without departing from its scope.

We claim:

1. A process for preparing a hydrocarbon lubricating oil that is miscible with a fluorochlorinated hydrocarbon refrigerant at low temperatures which comprises alkylating a mixture of aromatic hydrocarbons consisting predominantly of at least two different hydrocarbons from the group consisting of methyl ethyl benzene, dimethyl

ethyl benzene, trimethyl benzene, and tetramethyl benzene, with a polymer of propylene having 9 to 15 carbon atoms, in the presence of an alkylation catalyst, the weight ratio of the said mixture of aromatic hydrocarbons to propylene polymer being in the range of from 1:1 to 7:1.

5 2. A process as defined by claim 1 in which the alkyl aromatic hydrocarbon mixture is a petroleum fraction distilling between 170 and 325° C., 50% distilling at 180° C., and of mean molecular weight 136 and density 0.905.

10 3. A process as defined by claim 1 wherein the catalyst is selected from the group: sulphuric acid and a Lewis acid.

4. A process as defined by claim 1 wherein said weight ratio is within the range of 3:1 to 5:1.

15 5. A process as defined by claim 1 wherein said mixture of aromatic hydrocarbons is a mixture of methyl ethyl benzene and tetramethyl benzene.

6. A process as defined by claim 1 wherein said mixture 20 of aromatic hydrocarbons is a mixture of dimethyl ethyl benzene and tetramethyl benzene.

7. An improved refrigerant-lubricant composition for use in a compression refrigeration apparatus which comprises a major proportion of a fluorochlorinated hydrocarbon refrigerant and from 1 to 10 weight percent of the 25 hydrocarbon lubricating oil prepared by the process of claim 1.

#### References Cited

##### UNITED STATES PATENTS

- 30 3,092,981 6/1963 Begeman et al. ----- 252-68  
3,169,928 2/1965 Herold ----- 252-68  
3,214,462 10/1965 Swenson et al. ----- 260-671

##### FOREIGN PATENTS

- 35 664,095 1/1952 Great Britain.  
665,058 1/1952 Great Britain.  
666,209 2/1952 Great Britain.

DELBERT E. GANTZ, Primary Examiner.

40 C. R. DAVIS, Assistant Examiner.

U.S. CL. X.R.

252-68